

[54] PLATED METALLIC CATHODE

[75] Inventors: **Han C. Kuo; Ronald L. Dotson; Kenneth E. Woodard, Jr.**, all of Cleveland, Tenn.[73] Assignee: **Olin Corporation**, New Haven, Conn.

[\*] Notice: The portion of the term of this patent subsequent to Jul. 5, 1994, has been disclaimed.

[21] Appl. No.: **812,210**[22] Filed: **Jul. 1, 1977****Related U.S. Application Data**

[63] Continuation-in-part of Ser. No. 660,847, Feb. 24, 1976, Pat. No. 4,033,837.

[51] Int. Cl.<sup>2</sup> ..... **C25B 1/34; C25B 11/04**[52] U.S. Cl. ..... **204/290 R; 204/43 T**

[58] Field of Search ..... 204/293, 43 S, 290 R, 204/291

[56] **References Cited****U.S. PATENT DOCUMENTS**3,947,331 3/1976 Kinh et al. ..... 204/37 R  
4,033,837 7/1977 Kuo et al. ..... 204/98**OTHER PUBLICATIONS**

Malachowski, Zesz. Nauk. Politech. Slask. Chem. No. 65, 235, 236 (1973).

*Primary Examiner*—F.C. Edmundson  
*Attorney, Agent, or Firm*—Bruce E. Burdick; Donald F. Clements; Thomas P. O'Day[57] **ABSTRACT**

A highly conductive and corrosion resistant low hydrogen overvoltage cathode. The cathode comprises a copper substrate plated with an alloy of nickel, vanadium, and molybdenum.

**9 Claims, 2 Drawing Figures**

FIG-1



FIG- 2



## PLATED METALLIC CATHODE

This application is a continuation-in-part of Applicant's copending application Ser. No. 660,847 filed Feb. 24, 1976, now U.S. Pat. No. 4,033,837 issued July 5, 1977.

This invention relates generally to a cathode for an electrolytic cell, and more particularly, to a plated metallic cathode for use in such cells.

One of the largest costs in the operation of electrolytic cells is that of electrical energy. Consequently, efforts have been made to reduce the working voltage of the cell. One of the components contributing to the working voltage is the overvoltage at the cathode. In the case of a cell used for the electrolysis of alkali metal chloride solutions, for example, this component is referred to as hydrogen overvoltage.

Previously, cathodes have been constructed of various metals such as low-carbon steel, titanium, nickel, chromium, copper, iron, tantalum, and the like, and alloys thereof, especially stainless steel and other chromium steels, nickel steels, and the like. For a given structural configuration, current density, temperature, and electrolyte, each of these metals when used as a cathode will possess a given overvoltage.

In an article published in *Zeszyty Naukowe Politechniki Śląskiej, Chemia* No. 65, pp. 235 and 236, 1975 (Poland), by Andrzej Malachowski, there is disclosed an electrode having a reduced hydrogen overvoltage. The electrode disclosed in the article comprised a steel substrate plated with a nickel, molybdenum, vanadium alloy. Although the Ni-Mo-V plated steel electrode does have a reduced overvoltage, it has been found to be prone to corrosion, even to the extent that the plating will peel off after a few weeks when the potential is removed.

It is an object of the present invention to provide an improved cathode which has a relatively low hydrogen overvoltage.

It is a further object of the present invention to provide an improved cathode having a relatively low hydrogen overvoltage and improved corrosion resistance.

The above objects may be accomplished, according to the preferred form of the invention, through the provision of a cathode comprising a copper substrate plated with an alloy of nickel, molybdenum and vanadium in a complexing agent containing plating bath having a pH greater than about 9.0.

A better understanding of this invention may be had by reference to the following detailed description and to the accompanying drawing in which FIGS. 1 and 2 are graphs plotting the polarization potential against various current densities for various plated and unplated cathodes.

More specifically, it is contemplated that the cathode structure may be of any shape suitable for the intended purpose. For example, the cathode of the present invention may comprise a plate, a rod, a foraminous structure, or mesh of any shape well known in the art.

The cathode is fabricated from a copper substrate to which is applied a plating of an alloy of nickel, molybdenum and vanadium. The percent by weight of the various alloys in the plating may be as follows: nickel, 80 to 90; vanadium, 0.2 to 1.5; and molybdenum, 10 to 20. The thickness of the plating may be in the order of 2 to 30 microns. Preferably, the thickness is in the order of about 20 to 25 microns.

The nickel, molybdenum, vanadium plating is preferably electrodeposited on the copper substrate using a Watt's bath with the addition of small amounts of a vanadium and molybdenum in a form that will provide a source of ions to be deposited by discharge in an aqueous solution. The bath may be an aqueous solution of nickel sulfate in the amount of 240 to 340 g/l (grams per liter), nickel chloride in the amount of 30 to 60 g/l, and boric acid in the amount of 20 to 40 g/l. The molybdenum and vanadium ion source may be sodium molybdate in the amount of 0.2 to 2.0 g/l and vanadium sulfate in the amount of 0.2 to 0.8 g/l. Other sources of the vanadium and molybdenum ion may be used.

Prior to immersing the copper substrate in the bath, the surface of the substrate should be cleaned. This can be accomplished by conventional techniques well known in the art for cleaning preparatory to nickel plating. For example, the copper substrate may be etched in a solution containing 10 to 40% volume parts sulfuric acid having a concentration of 97%  $H_2SO_4$  by weight, and 5 to 20 volume parts nitric acid having a concentration of 71%  $HNO_3$  by weight and 40 to 85 volume parts water for about 5 to 15 minutes at room temperature. Alternatively, it may be cathodically cleaned in a caustic solution of 10 to 20 weight parts sodium hydroxide and 80 to 90 weight parts water at room temperature at 20 to 80  $ma/cm^2$  for about 5 to 10 minutes. After either of the above operations, the copper substrate should be rinsed with deionized water. Prior to immersing the copper substrate into the plating bath, it may be immersed in a solution of about 10 volume parts sulfuric acid having a concentration of 97%  $H_2SO_4$  by weight, about 10 volume parts hydrochloric acid having a concentration of 37%  $HCl$  by weight, and about 80 volume parts water, room temperature, for 10 to 40 seconds and then rinsed with deionized water.

After cleaning, the copper cathode structure may be immersed in the above described plating bath. The bath may have a pH of 3.5 to 5.5 and be at a temperature of 20° to 45° C. The plating current density may be 20 to 80  $ma/cm^2$ . The plating operation may continue for 15 to 30 minutes or until a suitable layer of alloy material has been deposited.

The resulting product is a cathode having a copper substrate with a plating of about 80 to 90% by weight nickel, about 0.2 to 1.5% by weight vanadium, and about 10 to 20% by weight molybdenum.

As an alternative to the above-described modified Watts bath plating solution, a plating bath having a pH of about 9.0 to about 11.0 and a temperature of 20° to 45° C can be used. The plating current density can be 20 to 80  $ma/cm^2$  and the plating operation can continue for 15 to 30 minutes or until a suitable layer of alloy material has been deposited. This alternative plating bath solution has the following composition: nickel sulfate 50 to 100 g/l, nickel chloride 5-30 g/l, sodium molybdate 1-20 g/l, vanadium sulfate 0.1-1.0 g/l and a tartrate or citrate compound 50-100 g/l. The tartrate or citrate compound would preferably be sodium citrate, sodium tartrate, ammonium citrate, ammonium tartrate so that a common cation (i.e.  $Na^+$  or  $NH_4^+$ ) is added rather than some contaminant cation which might have harmful effects. The pH of the plating solution can be adjusted by addition of either ammonium hydroxide or sodium carbonate so as to fall within the range of about 9.0 to about 11.0. Ammonium hydroxide can serve both as a pH raiser (i.e. base) and as a nickel complexing agent.

The cathodes of the present invention show lower hydrogen overvoltages at various current densities as compared with bare copper, bare mild steel, and bare stainless steel 308. In addition, the plated copper cathode of the present invention shows improved corrosion resistant properties as compared to a mild steel plated with the same alloy.

The cathode of this invention is particularly useful in chlor-alkali electrolytic cells. However, it is contemplated that it may also be used in the electrolysis of water.

The following examples are presented to better define the invention without any intention of being limited thereby. All parts and percentages are by volume at room temperature unless otherwise indicated.

#### EXAMPLE I

A  $\frac{1}{8}$  inch diameter copper rod was etched for 10 minutes in a mixture of 20 volume parts of analytical grade sulfuric acid having a concentration of 97%  $H_2SO_4$  by weight, 5 volume parts of analytical grade nitric acid having a concentration of 71%  $HNO_3$  by weight, and 75 volume parts water. After etching, the copper rod was rinsed in deionized water. Prior to immersing in the plating bath, the copper rod was dipped in a solution of 10 volume parts of analytical grade sulfuric acid having a concentration of 97%  $H_2SO_4$  by weight, 10 volume parts of analytical grade hydrochloric acid having a concentration of 37%  $HCl$  by weight for about 30 seconds. After dipping, the copper rod was rinsed in deionized water. The copper rod was placed in a plating bath comprising 300 g/l nickel sulfate, 60 g/l nickel chloride, 20 g/l boric acid, 0.6 g/l sodium molybdate, and 0.4 g/l vanadium sulfate. The bath was run at  $25^\circ \pm 2^\circ C$  at a current density of  $30 \text{ mA/cm}^2$  for 10 minutes and at  $60 \text{ mA/cm}^2$  for an additional 10 minutes.

A  $\frac{1}{8}$  inch diameter steel rod and a  $\frac{1}{8}$  inch diameter stainless steel rod were etched in a solution of 10 volume parts analytical grade sulfuric acid having a concentration of 97%  $H_2SO_4$  by weight and 90 volume parts water for 10 minutes. After rinsing with deionized water, the two steel rods were anodically cleaned in a caustic solution of 10 volume parts sodium hydroxide and 90 parts water for 5 minutes at  $50 \text{ mA/cm}^2$  (milliamps per square centimeter) after which they were washed in deionized water. Prior to immersion on the plating bath, the rods were dipped in a solution of 10 volume parts of analytical grade sulfuric acid having a concentration of 97%  $H_2SO_4$  by weight and 90 volume parts water for about 30 seconds. The steel rods were then placed in the bath and plated as described above in connection with the copper rod.

Each of the plated rods were operated as a cathode with varying current densities in a solution of 13 weight parts  $NaOH$ , 15 weight parts  $NaCl$ , and 72 weight parts water at  $25^\circ C$  and the polarization potential determined for various current densities using a saturated calomel electrode. A similar procedure was used to determine the polarization potential of  $\frac{1}{8}$  inch diameter bare copper, bare mild steel, and bare stainless steel rods in the same solution.

The results of various readings of the rods are plotted on the graph of FIG. 1, which shows the polarization potential in volts versus a saturated calomel electrode plotted along the ordinate in decreasing magnitude and the current density in  $KA/M^2$  (kiloamps per square meter) plotted along the abscissa in increasing magnitude. Thus the current at the upper portion of the

graphs have a less negative polarization potential. The polarization potential gives a direct indication of relative overvoltage as overvoltage is equal to polarization potential minus the reversible potential.

As the graph of FIG. 1 shows, the polarization potential and thus the overvoltage, of the Ni—V—Mo plated copper rod cathode is slightly lower than that of the mild steel rod plated with the same alloy and on the order of 100 mv lower than that of the same alloy plated on stainless steel 308 rod. Also, the polarization potential of the plated copper rod cathode is on the order of about 280 mv lower than that of a rod of bare mild steel and an even greater reduction is shown with respect to a rod of bare copper.

#### EXAMPLE II

Two  $\frac{1}{8}$  inch diameter copper rods, which had been etched, rinsed, and dipped as set forth in Example I were plated in a bath of the same composition and temperature as set forth in Example I. One rod was plated for 20 minutes at  $30 \text{ mA/cm}^2$  and the other for 15 minutes at  $60 \text{ mA/cm}^2$ . Both rods were used as a cathode at various current densities in a 36% by weight caustic solution at  $24^\circ C$  and the polarization potential was determined using a saturated calomel electrode. An unplated mild steel  $\frac{1}{8}$  inch diameter rod was also tested in the same solution.

The results of various readings were plotted on the graph of FIG. 2 with the polarization potential in volts versus a saturated calomel electrode plotted along the ordinate in decreasing magnitude and current density in  $KA/M^2$  plotted along the abscissa in increasing magnitude. The polarization potential and thus the hydrogen overvoltage of the two plated copper rods is about the same and about 220 mv lower than that of bare mild steel.

#### EXAMPLE III

Several Ni—Mo—V plated copper and mild steel rods of  $\frac{1}{8}$  inch diameter were plated according to the procedures set forth in Examples I and II. The plated electrodes were put into a 25% brine solution having a  $pH=6$  for an accelerated corrosion test without polarization. Within 3 to 5 days visible pits started to form on the plated steel surface and the coatings peeled off in many instances after two weeks immersion time. No visible corrosion was observed on the plated copper rods after 3 weeks and no coatings peeled off.

#### EXAMPLE IV

A  $\frac{1}{8}$  inch diameter copper rod was plated with the Ni—Mo—V alloy according to the procedure set forth in Example I. The plated copper rod was operated in a small brine electrolytic cell as a cathode at  $4 \text{ KA/m}^2$  for about 5 weeks. During that time, no visible corrosion was observed and the hydrogen overvoltage did not change.

As indicated by the polarization potential, the hydrogen overvoltage of the Ni—Mo—V plated copper cathode is substantially lower than that of bare copper, bare mild steel, and bare stainless steel. Although in some cases, the overvoltage of Ni—Mo—V plated mild steel compared favorably with that of similarly plated copper, the plated copper cathode exhibited better corrosion resistant properties.

## EXAMPLE V

Three copper rods of 0.25 diameter were plated at a current density of 40 milliamperes per square centimeter for 10 minutes at  $26^\circ \pm 2^\circ$  C in a bath having the following composition:

| INGREDIENT               | CONCENTRATION | 10 |
|--------------------------|---------------|----|
| Nickel Sulfate           | 50 g/l        |    |
| Nickel Chloride          | 5 g/l         |    |
| Sodium Molybdate         | 15 g/l        |    |
| NH <sub>4</sub> OH (28%) | 200 ml/liter  |    |

Prior to the plating of each of the three rods, a varying amount of vanadium sulfate was added to the plating solution and the hydrogen overvoltage ("HO") of the copper rods so plated was then tested at a current density of 2 KA/m<sup>2</sup> in an aqueous solution of 200 g/l NaOH at  $80^\circ$  C with the following results:

| Plated Copper Rod Number | VSO <sub>4</sub> Concentration In Plating Solution | HO     | 15 |
|--------------------------|----------------------------------------------------|--------|----|
| 1                        | 0.0 g/l                                            | 404 mv |    |
| 2                        | 0.2 g/l                                            | 284 mv |    |
| 3                        | 0.4 g/l                                            | 224 mv |    |

The hydrogen overvoltage of aged steel in the same aqueous solution of 200 g/l NaOH is found to be about 450 mv.

## EXAMPLE VI

A 0.25 inch diameter copper rod is plated at a current density of 40 ma/cm<sup>2</sup> for 10 minutes at  $40^\circ$  C in a bath having the following composition:

| INGREDIENT         | CONCENTRATION | 35 |
|--------------------|---------------|----|
| Nickel Sulfate     | 79.0 g/l      |    |
| Nickel Chloride    | 23.8 g/l      |    |
| Sodium Molybdate   | 4.0 g/l       |    |
| Vanadium Sulfate   | 0.5 g/l       |    |
| Ammonium Sulfate   | 73.6 g/l      |    |
| Ammonium Hydroxide | *             |    |

\*sufficient to achieve pH of 9.8

The hydrogen overvoltage of the plated sample in 200 g/l NaOH aqueous solution at  $80^\circ$  C at a current density of 2 KA/m<sup>2</sup> is about 195 mv.

An expanded copper mesh of 50 cm<sup>2</sup> is plated in the above bath with the same plating solution at the same plating conditions and shows the same hydrogen overvoltage under the same test conditions.

## EXAMPLE VII

A 0.25 inch diameter copper rod was plated at a current density of 40 ma/cm<sup>2</sup> for 10 minutes at  $26^\circ \pm 2^\circ$  C in a bath having the following composition:

| INGREDIENT       | CONCENTRATION                 |
|------------------|-------------------------------|
| Nickel Sulfate   | 79.0 g/l                      |
| Nickel Chloride  | 23.8 g/l                      |
| Sodium Molybdate | 4.0 g/l                       |
| Vanadium Sulfate | 0.3 g/l                       |
| Sodium Citrate   | 60.0 g/l                      |
| Sodium Carbonate | As needed to obtain pH of 9.0 |

The hydrogen overvoltage when tested at a current density of 2 KA/m<sup>2</sup> at  $80^\circ$  C in a 200 g/l NaOH aqueous solution was 160 mv.

What is claimed is:

1. A cathode for use in electrolytic cells comprising:
  - (a) a copper substrate,
  - (b) a plating on said copper substrate,
  - (c) said plating being an alloy of vanadium, molybdenum and nickel,
  - (d) wherein said plating is applied to said cathode structure by electrodeposition using a bath comprising an aqueous solution of the following:

|                  |               |
|------------------|---------------|
| nickel sulfate   | 50 to 100 g/l |
| nickel chloride  | 5 to 30 g/l   |
| sodium molybdate | 1 to 20 g/l   |
| vanadium sulfate | 0.1 to 1 g/l  |

2. The cathode of claim 1, wherein said bath has a pH of about 9.0 to about 11.0 and a nickel complexing agent.

3. The cathode of claim 2, wherein said complexing agent is selected from the group consisting essentially of ammonium hydroxide, ammonium citrate, ammonium tartrate, sodium citrate and sodium tartrate.

4. The cathode of claim 2, wherein the concentration of said nickel complexing agent in said bath is about 50-100 g/l.

5. The cathode of claim 3, wherein said nickel complexing agent consists essentially of ammonium hydroxide.

6. The cathode of claim 5 wherein the concentration of said ammonium hydroxide in said bath is about 200 ml/l.

7. The cathode of claim 3, wherein said nickel complexing agent consists essentially of sodium citrate and sodium tartrate and sufficient sodium carbonate is present in said bath to produce a pH within the range of about 9.0 to about 11.0.

8. The cathode of claim 3, wherein said nickel complexing agent consists essentially of one of ammonium citrate and ammonium tartrate and ammonium hydroxide is added to said bath in a sufficient quantity to raise the pH of said bath to within the range of about 9.0 to about 11.0.

9. The cathode of claim 2, wherein the current density during said application of said plating is within the range of from about 20 ma/cm<sup>2</sup> to about 80 ma/cm<sup>2</sup>.

\* \* \* \* \*